

193 Patented Sept. 1, 1936

## UNITED STATES PATENT OFFICE

2,052,557

## TREATMENT OR PRODUCTION OF CELLULOSE DERIVATIVE MATERIALS

Henry Dreyfus, London, England

No Drawing. Application May 26, 1930, Serial  
No. 455,969. In Great Britain July 9, 1929

3 Claims. (Cl. 18—54)

This invention relates to new or improved processes for the weighting or mordanting of materials made of or containing cellulose acetate or other cellulose esters or ethers, for example cellulose formate, cellulose propionate, cellulose butyrate, or methyl, ethyl or benzyl cellulose.

It is well-known that the incorporation of metallic radicles in materials made of or containing cellulose esters or ethers has presented considerable difficulties. In the case of weighting and mordanting metal radicles these difficulties have been overcome by treatment of the filaments, threads, yarns, ribbons, woven, knitted or other fabrics, or other materials with solutions 10 of salts of the weighting or mordanting metals under such conditions that swelling of the cellulose derivative occurs. The weighting or mordanting metal solution may be applied in such concentrations or under such conditions that it 15 itself constitutes a swelling agent for the cellulose derivative, or alternatively a swelling agent may be incorporated in the solution or may be applied to the material prior to the mordanting or weighting metal solution. On the other hand 20 combinations of these methods may be employed. The mordanting or weighting metal may be fixed in the material by a previous or subsequent treatment with a suitable precipitant for the metal salt, for example phosphates, silicates, tannic acid 25 or tannates, or even water containing a little alkali in solution. Numerous prior specifications 30 of British Celanese Limited, R. Clavel and myself describe such processes and these specifications instance as examples of suitable mordanting and 35 weighting metals, aluminum, chromium, iron, tin, zinc, tungsten and bismuth.

I have now found that a very effective mordanting or weighting of such materials may be achieved by incorporating either a precipitant or 40 a compound of the mordant or weighting metal in the spinning solution used in the manufacture of the filaments or other products and treating the products, either subsequent to their production or continuously with or in the course of their production, with the mordant or weighting metal 45 compound or precipitant as the case may be.

According to the present invention therefore 50 filaments, threads, yarns, ribbons, fabrics or other materials made of or containing cellulose acetate or cellulose esters or ethers are mordanted or weighted by precipitating in the materials insoluble mordanting or weighting metal compounds, the mordanting or weighting metal salt or the 55 precipitant necessary for the formation of the

insoluble mordanting or weighting compound being incorporated in the spinning solutions used for the manufacture of the materials.

In the case of incorporating the precipitant, e. g. tannic acid, in the spinning solutions the mordanting or weighting metal preferably is applied to the finished materials, or to the materials continuously with their production, under such conditions that swelling of the cellulose derivative occurs. The principles employed in U. S. 10 Patents Nos. 1,631,062, 1,806,048, 1,821,464, 1,817,741 and 1,867,658 etc. may thus, for example, be used to apply the mordant or weighting metal radicles. I prefer however to incorporate the mordanting or weighting metal compound itself in the spinning solutions and subsequently to apply the precipitant. As examples of suitable mordanting or weighting metal salts which may be incorporated in the spinning solutions the following may be instanced: stannic chloride, stannic thiocyanate, ferric chloride, ferric thiocyanate, aluminium thiocyanate, zinc chloride, and chromium thiocyanate. The proportion of weighting or mordanting metal relative to the cellulose acetate or other cellulose derivative may be 25 varied as desired. In the case of mordanting, an addition of one to two percent of the mordant metal salt on the cellulose acetate or other cellulose derivative is usually sufficient, while, in the case of weighting, proportions of 10 to 20% or upwards 30 may be used. The precipitant may be applied either to the finished materials in thread, yarn, fabric or other form or may be applied to the filaments, threads or yarns during or continuously with their production. For example, the 35 filaments coming from a dry spinning cell may be carried directly into an aqueous bath containing di-sodium hydrogen phosphate or containing water having alkali in solution. Water itself may be used as the fixing agent or precipitant, especially in the case of mordant metals, but it is preferable to have a small amount of alkali, such as ammonia or soda ash, in solution. Again, in the case of wet spinning, the precipitant may be incorporated in the precipitating bath or in a subsequent treatment bath. For the purpose of wet spinning I find that the direct acetylation or other 40 esterification solutions, with or without ripening or further treatment, obtained according to British Patents Nos. 308,322, 308,323 and 309,201 and U. S. Patents Nos. 1,936,586, 1,950,663 and 1,911,069, are particularly suitable. These direct acetylation or esterification solutions already contain metallic radicles, for example zinc, iron and 45

50

55

tin, and may be spun into precipitating baths containing a precipitant for the metal salt. Mineral acidity or excessive mineral acidity due for example to the use of hydrochloric acid in the esterification or ripening, may be neutralised if desirable or requisite prior to spinning, for instance by adding sodium acetate to the solutions.

The following examples show the best methods known to me for carrying the invention into effect, 10 but they are not to be considered as limiting the invention in any way:—

*Example 1*

To a 25% solution of cellulose acetate in acetone 15 12% of stannic thiocyanate calculated on the cellulose acetate is added, and the solution is then spun into filaments by the dry spinning process. The yarn obtained, with or without intermediate washing, is treated for about half an hour at 40° 20 C. in a 12% aqueous solution of disodium hydrogen phosphate. Such treatment may be applied to the goods in the form of hanks or in the form of knitted, woven or other fabrics or in any other desired form. The goods may be subsequently 25 soaped in a bath containing 2½ grams per litre of soap, rinsed in soft water and dried.

*Example 2*

A spinning solution is made up with the following ingredients, the parts being by weight:—

|                    | Parts     |
|--------------------|-----------|
| Cellulose acetate  | 25        |
| Ferric thiocyanate | 0.75      |
| Acetone            | 74.25     |
|                    | <hr/> 100 |

The solution is then spun into filaments, and the yarn with or without intermediate washing and 40 continuously with production or in a separate operation in the form of hanks, fabrics or in any other form, treated with a solution of soda ash of about 5° Tw. at 30–35° C. The materials may subsequently be rinsed in soft water.

*Example 3*

An acetylation solution obtained according to Example 1 of British Patent No. 309,201 is treated with dilute acetic acid (about 40%) to remove excess of acetic anhydride and an aqueous solution of sodium acetate added until mineral acidity is removed. The solution thus obtained is heated to

about 50–60° C. and maintained at this temperature until a test sample shows that acetone solubility has been reached. The solution thus obtained is spun into a coagulating bath containing 10–15% aqueous acetic acid. The fixation of the 5 iron mordant may be effected by carrying the filaments into a subsequent treatment bath consisting of soda ash as described in the preceding example, or such a treatment may be applied discontinuously from the spinning operation. Alternately 10 sodium phosphate may be added to the coagulating bath itself to effect the desired fixation.

The materials mordanted or weighted according to the present invention may be coloured by any suitable processes and with any suitable colouring matters, for example with mordant dyestuffs. As is already known materials made of or containing cellulose esters or ethers which have been weighted have an affinity for the direct cotton dyestuffs and may therefore be dyed or coloured with such dyestuffs. If compatible therewith, the mordant or other dyestuffs may be incorporated in baths used for fixing or precipitating the mordant or weighting metals.

What I claim and desire to secure by Letters 25 Patent is:—

1. In the manufacture of extruded products comprising organic derivatives of cellulose by spinning processes, the steps of introducing a mordant or weighting metal compound into the 30 spinning solution, extruding said solution into a setting medium, fixing the metal in the extruded products by the application of a suitable fixing agent, and simultaneously coloring the products.

2. In a process for the manufacture of materials comprising organic derivatives of cellulose by spinning processes, the steps of introducing a mordant metal compound into the spinning solution, extruding the solution, and coagulating the same in a medium adapted simultaneously to fix 40 the metal in the coagulated materials and to color the materials.

3. In a process for the manufacture of materials comprising organic derivatives of cellulose by spinning processes, the steps of introducing a 45 mordant metal compound into the spinning solution, extruding the solution, and coagulating the same in a medium adapted simultaneously to fix the metal in the coagulated materials and, in conjunction with the mordant, to color the materials. 50

HENRY DREYFUS.